

I. S. FRANKLIN.

CLOSET SEAT AND METHOD OF MAKING THE SAME.

APPLICATION FILED SEPT. 23, 1918.

1,315,488.

Patented Sept. 9, 1919.



Fig. 2.

Fig. 3.

Fig. 4.

Fig. 1.

Fig. 5

Fig. 6.

Inventor:  
Ira S. Franklin  
By Knott & Son, Quincy, Mass  
Attorneys

# UNITED STATES PATENT OFFICE.

IRA S. FRANKLIN, OF BOSTON, MASSACHUSETTS.

## CLOSET-SEAT AND METHOD OF MAKING THE SAME.

1,315,488.

Specification of Letters Patent.

Patented Sept. 9, 1919.

Application filed September 23, 1918. Serial No. 255,244.

To all whom it may concern:

Be it known that I, IRA S. FRANKLIN, a citizen of the United States, residing at Boston, in the county of Suffolk and State of Massachusetts, have invented new and useful Improvements in Closet-Seats and Methods of Making the Same, of which the following is a specification.

This invention has for its object to provide a relatively inexpensive and at the same time rigid and practically non-breakable closet seat, adapted to be finished externally by buffing and varnishing, and free from joints or cracks liable to separate and receive disease germs.

The invention is embodied in the improved seat and in the method of making the same hereinafter described and claimed.

Of the accompanying drawings forming part of this specification:

Figure 1 represents in plan the layers of which the seat is made, said layers being separated from each other.

Fig. 2 is a section of line 2—2 of Fig. 1.

Fig. 3 is a perspective view of a seat formed by assembling said layers and cementing them together.

Fig. 4 is a section of line 4—4 of Fig. 3.

Fig. 5 is a view similar to Fig. 4, showing the completed seat.

Fig. 6 is a plan view of a layer formed as a member of an open-front seat.

The same reference characters indicate the same parts in all the figures.

In carrying out my invention, I cut by a die from suitable absorbent fibrous sheet material, such as paper board used for book bindings, and preferably from one-eighth (1/8) to three sixteenths (3/16) of an inch in thickness, a plurality of seat-shaped layers 12, each of which preferably has an opening 13 formed by the die which forms the margin of the layer. The layers are of identical form, so that, when assembled as indicated by Fig. 3, they form a seat, or seat-body of suitable thickness, any desired number of layers being employed. Before assembling the layers, I coat their proximate surfaces with any suitable adhesive composition adapted to penetrate said surfaces to a depth of at least one-sixteenth of an inch (1/16). The adhesive composition may be composed of one pound of dried glue softened by cold water, and then converted into a somewhat thick and viscous solution by boiling water, four-fifths of an ounce of glycerin, and two-

thirds of an ounce of either bichromate of potash or bichromate of soda. The layers are then assembled, with their openings coinciding, while the adhesive is soft. The assemblage of layers is then subjected to pressure, which is maintained until the adhesive sets or solidifies by drying, a laminated seat or seat-body being thus formed, which is rendered rigid by the adhesive composition permeating considerable portions of the layers. The seat is then finished, preferably by the operations next described.

The margin of the seat opening is suitably beveled or tapered by a trimming tool.

The external surfaces of the seat are next buffed by sand-paper or any other suitable abrading instrumentality.

To the buffed surfaces is applied a water-proof and acid-proof coating, composed of a hard-drying

pasty composition adherent to the abraded surfaces, the coating being adapted to be buffed and varnished.

This composition may consist of one pound of dried glue converted into a thinner solution than that above described, adapted to take up a powder

and thus form a semi-liquid composition of the consistency of paste, four-fifths of an ounce of glycerin, two-thirds of an ounce of bichromate of potash or bichromate of soda

and a sufficient quantity of powdered talc to form a pasty composition adapted to be applied and spread smoothly by a brush.

The nature of the said composition is such that the coating formed thereby adheres firmly to the surfaces to which it is applied.

The coating is indicated by the heavy black line 14 in Fig. 5. The coating 14 is allowed to solidify by drying, and is finally dressed or finished in any suitable way, as by first

buffing and then varnishing the coating.

The composition may contain coloring matter suitable for imparting the color of mahogany to the coating 14, and the varnish may be similarly colored.

The chief object of the coating 14 is to enable the external surfaces of the seat to be finished to closely resemble mahogany or other wood.

The powdered material gives body to the coating and enables it to be buffed without exposing the material of the layers 12, the buffed and varnished surface of the coating being separated by the body of the coating from the surfaces of the layers which back and support the coating.

The layers 12 may be cut from sheet material by a die adapted to form only the mar-

gins of the layers, the seat opening being formed by a saw after the layers are assembled. I prefer to employ a sufficient number of layers to form a seat of about one and one-eighth inch (1 $\frac{1}{8}$ ") in thickness.

5 I am enabled by the described method to provide a seat which is relatively inexpensive, can be finished in any desired color, is adapted to repel moisture and acid, and is free from liability to shrink and swell and 10 form cracks.

As shown by Fig. 6, the openings 13<sup>a</sup> in the layers 12 may be open at one end, so that the seat may be of the open-front type.

15 The preferred mode of operation, including the step of providing each layer with an opening before the layers are assembled, enables the seat opening to be provided by the operation of assembling the layers, the expense of a subsequent opening-forming operation after the layers are assembled being avoided.

I claim:

20 1. The method of making a closet seat constituting a completed article of manufacture, which consists in forming a seat from a plurality of layers of fibrous sheet material coated with an adhesive which penetrates the surfaces thereof, the layers being assembled while the adhesive is soft, and subjected to pressure until the adhesive sets or solidifies by drying, and finishing the surfaces of the seat by buffing said surfaces, applying to the buffed surfaces a pasty water-proof and acid-proof coating adapted to be buffed and varnished, and including a hard-drying liquid adherent to and penetrating the said abraded surfaces and powdered material giving body to the coating, allowing said coating to solidify by drying, and finally buffing and varnishing said coating.

25 2. The method of making a closet seat constituting a completed article of manufacture, which consists in cutting out, from absorbent fibrous sheet material, a plurality of seat-shaped layers, coating said layers with an adhesive, which penetrates the surfaces thereof, assembling the layers, while the adhesive is soft, subjecting the assembled layers to pressure and maintaining the pressure until the adhesive sets or solidifies by drying, thus forming a rigid laminated seat, forming a tapered opening-margin in the seat, and then finishing the external surfaces of the seat by buffing said surfaces, applying to the buffed surfaces a pasty water-proof and acid-proof coating adapted to be buffed and varnished, and including a hard-drying liquid adherent to and penetrating the said abraded surfaces and powdered material giving body to the coating, allowing said coating to solidify by drying, and finally buffing and varnishing said coating.

30 3. As an article of manufacture, a closet seat comprising a plurality of layers of absorbent fibrous material, said layers being cemented together and absorbing a portion of the cement, and a rigid water-proof and acid-proof coating adherent to and covering the surfaces of said seat and having buffed and varnished surfaces separated by the coating from the surfaces of said layers which back the said coating.

35 In testimony whereof I have affixed my signature.

IRA S. FRANKLIN.